

May 23, 1939.

E. HOUDREMONT ET AL

2,159,086

MANUFACTURE OF HIGH SPEED STEELS

Filed Feb. 24, 1938

Work Material: Cr-Ni Steel of 100 Kg/mm<sup>2</sup> Tensile Strength  
Feed 1.4 mm.  
Depth of Cut 5.0 mm.  
Tool Dimensions 30 mm  $\phi$  x 300 mm long

|            | C    | Cr   | W    | V    | Mo   |
|------------|------|------|------|------|------|
| Steel with | 0.70 | 4.25 | 14.4 | 2.39 | —    |
| "          | 1.35 | 4.27 | —    | 4.69 | 3.25 |
| "          | 0.75 | 4.41 | —    | 2.51 | 3.10 |



Inventors  
Eduard Houdremont and  
Hans Schaefer

by Knight Bros  
Attorneys

## UNITED STATES PATENT OFFICE

2,159,086

## MANUFACTURE OF HIGH SPEED STEELS

Eduard Houdremont and Hans Schrader, Essen,  
Germany, assignors to Fried. Krupp Aktiengesellschaft,  
Essen-on-the-Ruhr, Germany

Application February 24, 1938, Serial No. 192,289  
In Germany September 30, 1937

3 Claims. (Cl. 75—126)

The present invention relates to steels intended for the manufacture of high speed machining tools. According to the invention such tools are made of steel alloys which contain from 0.6 to 5 1.0% carbon, from 1.0 to 6.0% chromium, from 1.0 to 6.0% molybdenum, and from 1.0 to 3.0% vanadium, the remainder substantially being iron with the normal impurities.

Steels of a composition as specified hereinbefore 10 although they contain only small percentages of alloying constituents are distinguished by a high efficiency in the chip-removing working of materials and can be equal in this respect even to the high alloy high speed tungsten steels or, under 15 favorable cutting conditions, even be superior to them. The best results are obtained by steels which contain the above alloying constituents within the following limits: Carbon from 0.6 to 1.0%, chromium from 3.0 to 6.0%, molybdenum from 2.0 to 4.0%, vanadium from 2.0 to 3.0%. So, for instance, as appears from the drawing, a steel 20 of a composition according to the invention containing 0.75% carbon, 4.41% chromium, 3.10% molybdenum, and 2.51% vanadium under cutting 25 conditions as stated in the drawing shows a longer time up to re-grinding than a high alloy steel containing 0.79% carbon, 4.25% chromium, 14.4% tungsten, and 2.39% vanadium. As will further be seen from the drawing, the time up to re- 30 grinding of this steel composed according to the

invention is even superior to that of a low alloy high speed steel containing 1.35% carbon, 4.27% chromium, 3.25% molybdenum, and 4.69% vanadium.

The efficiency of the new high speed steels can 5 be increased further by an addition of tungsten which amounts at least to 50% of the molybdenum content and comes within the limits of from 1.0 to 4.0%. Finally, the new steels may contain, 10 besides the constituents hereinbefore specified, up to 10.0% cobalt.

What we claim and desire to secure by Letters Patent is:

1. High speed steels composed of 0.6—1.0% carbon, 1.0—6.0% chromium, more than 1.0 and less than 5.0% molybdenum, 1.0—3.0% vanadium, remainder substantially all iron with the normal impurities.

2. High speed steels composed of 0.6—1.0% carbon, 3.0—6.0% chromium, 2.0 to 4.0% molybdenum, 20 2.0—3.0% vanadium, remainder substantially all iron with the normal impurities.

3. A cutting tool composed of high speed steel consisting of 0.6—1.0% carbon, 1.0—6.0% chromium, more than 1.0% and less than 5.0% molybdenum, 25 1.0—3.0% vanadium, the remainder substantially all iron with the normal impurities.

EDUARD HOUDREMONT.  
HANS SCHRADER.

30